

# UNITED STATES PATENT OFFICE.

HENRY C. P. WEBER, OF EDGEWOOD, PENNSYLVANIA.

## PROCESS OF PRODUCING METAL SUBSTANCES.

1,373,038.

Specification of Letters Patent. Patented Mar. 29, 1921.

No Drawing.

Application filed March 31, 1919. Serial No. 286,415.

To all whom it may concern:

Be it known that I, HENRY C. P. WEBER, a resident of Edgewood, in the county of Allegheny and State of Pennsylvania, have 5 invented a new and useful Improvement in Processes of Producing Metal Substances, of which the following is a specification.

The invention relates to a process of producing metals which are reducible only 10 with difficulty by the ordinary methods.

Metals which are readily reducible from their ores or compounds are ordinarily produced by heating an easily available ore or compound of the metal either alone or with 15 the addition of well known reducing agents, such for instance as carbon. The reduction of iron from its ores or compounds is a well known example. Certain metal ores or compounds however, do not lend themselves to 20 this simple treatment, and heretofore have been reduced only with difficulty or very incompletely. This is the case particularly with such metals as chromium, tungsten, molybdenum, uranium, titanium, columbium, tantalum, zirconium, cerium, thorium, vanadium, beryllium, and others. Such metals are ordinarily produced by treating a suitable compound thereof in a fused state, 25 at very high temperatures, with more powerful reducing agents, but this method is expensive and not very efficient. An exception is the so-called alumino-thermic process in which metallic aluminum in a fine state is used as the reducing agent, acting upon the 30 metallic compound in a state of either fusion or of incipient fusion, wherein the necessary temperature is furnished by the heat of the exothermic reaction. This, as well as the other process mentioned above, depends 35 upon the fact that the heat of formation of the compound to be reduced is less than that of the compounds formed in the reduction.

Attempts have also been made to produce these metals by electrochemical methods, 40 either at ordinary temperatures or in fused electrolytes. The availability or possibility of such methods depends upon the position of the metal to be deposited in the electrochemical series, or upon the combination of 45 this with the closely related factor of heat of formation.

In both of the above general methods the

difficulties rapidly increase as the metals to be reduced become more refractory. The electrochemical reduction of such metals, 55 such for instance as chromium, has not been successfully practised so far.

The improved process differs fundamentally from any of the prior methods in that it does not depend upon a reaction between 60 a liquid (fused solid) and a solid, or between two liquids (fused solids); nor does it depend essentially upon the heats of formation of the substances or compounds participating in the reaction, nor upon the position of the metals concerned in the electrochemical series. Thus, for instance, I can reduce chromium compounds by less electro-positive metals, such as copper or gold.

The reaction upon which the new process 70 depends is between a vapor which is a compound of the metal to be reduced, and another metal which may be either solid or in a fused condition and which is itself capable of being converted into a volatile compound 75 during the process. The availability of this process for reducing any metal substance or compound therefore depends mostly upon the volatilities of the gaseous compounds originally present and those formed during 80 the reaction, and their relative quantities, which may be controlled.

The process can well be illustrated for the production of chromium from its ores or compounds. An anhydrous volatile compound, such as chromium chlorid, is mixed 85 with another metal, such for instance as iron, capable of forming a volatile compound with the chromium by substitution.

The mixture is placed in a container which 90 can be evacuated and heated. The reaction sets in slowly even below red heat, and may be varied in speed and intensity by raising or lowering the temperature. 700° to 1200° centigrade is a very satisfactory range of 95 temperature. After a time (depending upon the temperature used) the chromium chlorid is reduced to metallic chromium,—a corresponding amount of iron having been converted into a volatile form, to-wit, iron 100 chlorid. Therefore at a moderate temperature there occurs a replacement,—the volatile chromium chlorid giving its chlorin to the reducing metal, to-wit, iron. The re-

action is between a vapor and a solid, or liquid, and the process is therefore not determined by either the heat of formation of the compound to be reduced or that of the compound formed during the reaction, nor by the position of the metal to be reduced in the electrochemical series, but depends upon the interaction between a vaporized compound of the metal to be reduced or produced with another metallic body which is also capable of forming a volatile compound during the reaction. In other words, the driving force of the process depends upon the different volatilities and the relative amounts, *i. e.*, "concentration" of the gaseous compounds, namely that originally present and the one which is formed as a result of the reaction.

The process is general and may be used for the production of any of the metals or metalloids heretofore enumerated, or even of other metalloids, such as silicon, as well as for the production of more easily reducible metals, such as cobalt, nickel and iron.

The reducing agent need not be iron, but can be any metallic substance capable of also forming a volatile compound during the reaction, such for instance as tin, zinc, lead or the like. Instead of the chlorid of the metal to be reduced or produced I may use other halogens, such as the fluorids, bromids, iodids, cyanids, or carbonyls, or in fact any form of vaporized compound which during the reaction will give up its volatile constituent to combine with the reducing metal or metallic substance.

By varying the conditions a wide variety of results can be obtained. Thus if the reducing metal (for instance iron) is added as a fine powder the reaction takes place rapidly and at lower temperatures, and the product (for instance chromium) is in powdered or granular form. If on the other hand solid pieces of reducing metal are used and the reaction is effected below the melting point of the metals, the reduced metal (for instance chromium) is deposited upon the reducing metal (for instance iron) as a coating. If an excess of the reducing metal is used and the temperature is held high enough, an alloy results (an alloy of iron and chromium under the conditions assumed). Furthermore, by simultaneously reducing the volatile compounds of two or more metals, an alloy can be produced. Thus if the chlorids of chromium and of nickel are simultaneously treated with the reducing metal in the form of a powder and at a low temperature, the resulting material will be a mixture of granulated or powdered chromium and nickel, which can be melted to form a nickel-chromium alloy; or if the chlorid of chromium and nickel be treated with an excess of iron and the temperature

maintained high, it will result in a nickel-chromium-iron alloy. Likewise if two or more reducing metals are used in excess, and the temperature maintained high, a triple alloy will also result, such for instance as reducing chlorid of chromium by the use of both iron and nickel in excess and at a high temperature, in which case a chromium-nickel-iron alloy is formed.

The process therefore is adapted not merely for producing difficultly reducible metals in pure form, but also for producing various alloys thereof with metals which are capable of acting as reducing metals in the process; and also for depositing a coating of the difficultly reducible metals on the surfaces of solid bodies of the reducing metals. For best securing the latter result the iron, steel or other solid metal which is to be coated is first cleaned and dried and then placed in a receptacle which preferably can be evacuated, is covered with a layer of anhydrous chromium chlorid, the receptacle then evacuated and gradually heated, whereupon by the decomposition described, ferric chloride is driven off and the chromium is deposited on the iron or steel body. The depth of the coating can be regulated by the temperature and by the length of time that the reaction is allowed to proceed.

It is not essential to the process that the volatile substances from which the metal is to be produced or deposited are present originally. Thus, the volatile compound (such as chromium chlorid) may be formed at one stage of the process, and the reducing agent (for instance iron) may be formed at another stage of the process,—the essential features of the process consisting in the presence of the reducible volatile compound (for instance chromium chlorid) at one stage of the process, and the subsequent reduction of the metal to metallic form from the volatile compound by another substance (for instance iron), whether these components are originally present or are produced during the course of the reaction. For instance, for the production of chromium, the commercial process would start with chromic oxid (or possibly chromite) which would be converted into the chlorid by means of carbon and chlorin in conjunction with each other according to the well known method, and this product would without further purification be subjected to the reducing action of the iron or other metal, for producing the metallic chromium.

The process can also be made continuous. For this purpose, in the case of chromium described, I add to the volatile chromium compound a reducing metal in sufficient quantity to displace a portion of the chromium. The chlorid formed from the reducing metal, say for instance ferric chlorid, is, by the addition of carbon or similar well

known reducing agent, again converted into metallic iron. The regenerated iron then reduces a fresh portion of the volatile chromium compound. In the same way the chloride driven off in reducing the ferric chloride to metallic iron can be recovered and used for converting a new portion of chromic oxide to the chloride. Thus limited quantities of reagents can by this manner of recovery, be used to reduce the chromium compound continuously, by merely supplying carbon or similar substance sufficiently to regenerate the reagents.

I do not wish to limit myself to the use of a vacuum as described. One purpose of the vacuum is to hasten the reaction. This however can be effected by the use of catalysts (fine powders) such as are commonly employed to accelerate gas reactions. Another purpose of the employment of a vacuum is to prevent access of interfering substances, such as water vapor, oxygen and the like during the reaction. This result however can be obtained by carrying on the process in an inert atmosphere, such as nitrogen. It is however desirable to carry out the process in the absence of oxygen or substances capable of yielding oxygen.

I claim:

- 30 1. The process of producing metals and metalloids of the character described, which consists in forming a sublimable compound of the metal substance to be reduced, and reducing such compound by another metallic substance capable of also forming a volatile compound during the reaction.
- 20 2. The process of producing metals and metalloids of the character described, which consists in forming a sublimable compound of the metal substance to be reduced, and heating the same in contact with a metallic substance capable of also forming a volatile compound and thereby reducing the metal of the first named vapor compound.
- 25 3. The process of producing metals and metalloids of the character described, which consists in forming a volatile compound of the metal substance to be reduced, reducing said compound by another metallic substance capable of also forming a volatile compound during the reaction, and during such reaction excluding interfering substances, such as oxygen and substances capable of yielding oxygen.
- 30 4. The process of producing metals and metalloids of the character described, which consists in forming a volatile compound of the metal substance to be reduced, reducing said compound by another metallic substance capable of also forming a volatile compound during the reaction, and adding a catalyst to hasten the reaction.
- 35 5. The process of producing metals and metalloids of the character described, which

consists in forming a volatile compound of the metal substance to be reduced, and reducing said compound by another metallic substance in a finely divided state and capable of also forming a volatile compound during the reaction, said reduction being carried on at a temperature below the melting point of the metal to be produced.

6. The process of producing alloys from metals and metalloid substances of the character described, which consists in forming volatile compounds of several metallic substances of the character described, and reducing said compounds by another metallic substance capable of also forming a volatile compound during the reaction.

7. The process of producing alloys from metals and metalloid substances of the character described, which consists in forming a volatile compound of a metal substance of the character described, and reducing the said compound by an alloy capable of also forming a volatile compound during the reaction.

8. The process of forming alloys from metals and metalloid substances of the character described, which consists in forming a volatile compound of a metal substance of the character described, and reducing said compound by an excess of another metallic substance capable of also forming a volatile compound during the reaction.

9. The process of producing metals and metalloids of the character described, which consists in reducing a volatile compound of the metal to be reduced by a substance capable of yielding during the process a metal or metalloid and which is capable of also forming a volatile compound during the reaction, said substance being heated to a temperature below its melting point.

10. The process of producing metals and metalloids which consists in forming a volatile compound of the metal to be produced, mixing the same with a metal capable of forming a volatile compound during the reaction and heating the mixture.

11. The process of producing metals and metalloids which consists in forming a volatile compound of the metal to be produced, mixing the same with a metal capable of forming a volatile compound during the reaction, placing the mixture under vacuum and heating the same.

12. The process of producing metals and metalloids which consists in forming a volatile compound of the metal to be produced, mixing the same with a metal capable of forming a volatile compound during the reaction and heating the mixture, the compound of said second metal being more volatile than the compound of said first metal.

13. The process of producing metals and metalloids which consists in forming a vola-

1. tile halid of the metal to be produced, mixing the same with a metal capable of forming a volatile halid during the reaction and heating the mixture, the halid of the 5 second metal being more volatile than the halid of said first metal.

14. The process of producing chromium which consists in forming chromium chlo-

rid, mixing the same with metallic iron and heating the mixture.

In testimony whereof, I have hereunto set my hand.

HENRY C. P. WEBER.

Witness:

ALICE A. TRILL.